

## 1

2,899,393

ELECTROLYTE CONTAINING A KETONE, AN  
ALKALINE EARTH METAL IODIDE, AND  
IODINE

John F. Schoeppe, Stuart L. Varner, and Frederick W. Herr, Grand Rapids, Mich., assignors to Lear, Incorporated, Grand Rapids, Mich., a corporation of Illinois

No Drawing. Application September 6, 1956  
Serial No. 608,178

9 Claims. (Cl. 252—62.2)

This invention relates to improvements in variable resistors of the types which comprise a closed receptacle containing a liquid electrolyte and electrodes having a surface adapted to contact said electrolyte and to provide a current-conducting path between said electrolyte and said electrodes. Such variable resistors include, but are not limited to, devices of the types shown in U.S. Patents Nos. 2,367,465; 2,376,377; and 2,387,313, sometimes referred to as liquid level switches. In this latter type of device, an air bubble within the aforesaid closed receptacle shifts about, upon tilting of the switch, to expose more or less of the electrode surface or surfaces whereby current through electrical circuits is varied. These and similar devices find use for a variety of purposes as, for example, in aircraft instruments for controlling the erection of vertical gyroscopes. The present invention is not concerned with any specific constructions of variable resistors. Rather, it relates to variable resistors of the broad type described in which, by reason of the utilization therein of the electrolytes hereafter described in detail, marked improvements in the operation and usefulness of said variable resistors is obtained.

A fully satisfactory electrolyte for use in variable resistors of the type here involved must satisfy a number of rigid and exacting criteria. Not only must it have good conductivity over a wide range of temperatures both above and below 0 degrees C. but it must also have long life and stability under the various conditions under which it is used. In addition, it must possess the characteristics of providing a nearly completely reversible reaction, it must not become too viscous under conditions of low temperature, it must be substantially inert to the electrodes and other materials with which it comes into contact, and it must not exhibit material physical instability due to thermal effects in the variable resistor. These and other desirable characteristics for a fully satisfactory variable resistor electrolyte have been appreciated by others but, so far, although various compositions have been suggested by others and used, there has been much left to be desired in the achievement of an ideal electrolyte.

The electrolytes which are used in accordance with the present invention represent a distinct improvement in at least most of the characteristics which are desired in such products over anything which, so far as is known, have heretofore been suggested or utilized. In general, the electrolytes comprise solutions, in ketones, of certain iodides, hereafter disclosed, and iodine. The ketones can be chosen from the aromatic, aromatic-aliphatic, aromatic-cycloaliphatic, cycloaliphatic, and aliphatic groups, it being particularly desirable to utilize the aliphatic ketones. Illustrative examples of such ketones are benzyl ketone, naphthyl ketone, benzyl ethyl ketone, cyclohexyl benzyl ketone, cyclohexyl isopropyl ketone, methyl isobutyl ketone, methyl amyl ketone, methyl ethyl ketone, diethyl ketone, methyl n-propyl ketone, n-amyl ketone, n-hexyl ketone, n-heptyl ketone, diisopropylketone, diisobutylketone, and diisobutylketone.

## 2

tone; and the like, as well as mixtures of any two or more thereof. Of particular utility are diisopropylketone and diisobutylketone and preferably mixtures thereof in which the ratio thereof, by volume, is from about 1 to 3 to about 3 to 1 and, more especially, from about 2 to 3 to about 3 to 2.

The iodides which are utilized in accordance with the present invention comprise those of calcium, magnesium, strontium and barium, namely, the alkaline earth metal iodides, and compatible mixtures thereof.

The proportions of the ingredients of the electrolyte can be varied, within reasonable limits, depending upon the particular results desired. In all cases, of course, the electrolyte is in liquid form and comprises a solution, in

- 15 a ketone or mixture of ketones, of the aforesaid iodide or iodides and iodine. In general, in each 100 ml. of electrolyte solution there should be present from about 3 to about 10 grams of said iodide and from about 8 to about 16 grams of iodine. A particularly preferred range of proportions comprises from about 4 to about 6 grams of said iodide and from about 10 to about 14 grams of iodine in each 100 ml. of electrolyte solution. It will be understood that, in general, an increase in the concentration of the said iodide will, up to a certain point depending upon 25 its solubility in the particular ketone or mixture of ketones utilized and depending upon the concentration of iodine, result in an increase in electrical conductivity of the electrolyte solution. However, the concentration of the said iodide should not be increased beyond the point 30 where the stability of the variable resistor is affected and where, at low temperatures under which the variable resistor may be required to function, the said iodide may crystallize or separate out of the electrolyte solution. In 35 the case of the iodine, an increase in its concentration up to a certain point will, in general, increase the conductivity of the electrolyte solution. Beyond that point, a further increase in the iodine concentration tends, in general, to have little effect at room temperatures and, in at least certain cases, the electrical conductivity is decreased at low 40 temperatures as, for example, temperatures of the order of -50 to -55 degrees C. The ratio of the said iodide to iodine in the electrolyte solution is quite variable. Excellent results, for example, are obtained with ratios of 1 to 6 and even higher. While, in general, and in the 45 particularly preferred embodiments of the invention, the iodine is advantageously present in amount greater than the amount of said iodide, the invention is not so limited. Satisfactory results can be obtained with the use of electrolytes in which the ketone solution contains both iodine 50 and said iodide and wherein the iodine is present in amount less than the amount of said iodide as, for instance, with ratios of 1 of iodine to 1 to 2 of said iodide.

The following examples are illustrative of electrolytes the use of which is variable resistors falls within the scope 55 of the invention. It will be understood that such examples are in no way limitative of the invention since numerous other electrolyte compositions can readily be prepared in the light of the guiding principles and teachings disclosed herein. Thus, for example, other ketones and 60 mixtures of various ketones can be utilized, and the proportions of the ingredients can be varied, within reasonable limits, as desired. The stated quantities of the aforesaid iodide and iodine represent the number of grams of each in 100 ml. of the electrolyte solution made by dissolving the said iodide and the iodine in the stated ketone or mixture of ketones.

## Example 1

Diisobutylketone.

|    |                |    |
|----|----------------|----|
| 70 | Calcium iodide | 6  |
|    | Iodine         | 13 |

## Example 2

|                         |    |
|-------------------------|----|
| Methyl n-propyl ketone. |    |
| Magnesium iodide        | 5  |
| Iodine                  | 11 |

## Example 3

|                    |   |
|--------------------|---|
| Diisopropylketone. |   |
| Srtronium iodide   | 4 |
| Iodine             | 7 |

## Example 4

|                   |   |
|-------------------|---|
| Diisobutylketone. |   |
| Barium iodide     | 5 |
| Iodine            | 9 |

## Example 5

|                   |                          |
|-------------------|--------------------------|
| Diisopropylketone | } equal parts by volume. |
| Diisobutylketone  |                          |
| Srtronium iodide  | 4                        |
| Calcium iodide    | 3                        |
| Iodine            | 10                       |

## Example 6

|                   |                          |
|-------------------|--------------------------|
| Diisopropylketone | } equal parts by volume. |
| Diisobutylketone  |                          |
| Magnesium iodide  | 5                        |
| Iodine            | 9                        |

## Example 7

|                   |                          |
|-------------------|--------------------------|
| Diisopropylketone | } equal parts by volume. |
| Diisobutylketone  |                          |
| Calcium iodide    | 5                        |
| Magnesium iodide  | 2                        |
| Iodine            | 11                       |

## Example 8

|                      |   |
|----------------------|---|
| Methyl ethyl ketone. |   |
| Srtronium iodide     | 6 |
| Iodine               | 6 |

## Example 9

|                         |   |
|-------------------------|---|
| Methyl isobutyl ketone. |   |
| Barium iodide           | 6 |
| Iodine                  | 5 |

## Example 10

|                         |   |
|-------------------------|---|
| Methyl n-propyl ketone. |   |
| Calcium iodide          | 7 |
| Iodine                  | 6 |

## Example 11

|                   |   |
|-------------------|---|
| Diisobutylketone. |   |
| Srtronium iodide  | 4 |
| Calcium iodide    | 3 |
| Iodine            | 7 |

## Example 12

|                    |   |
|--------------------|---|
| Diisopropylketone. |   |
| Barium iodide      | 5 |
| Iodine             | 7 |

For best results, certain precautions should be exercised in carrying out the preparation of the electrolyte solution. The iodide should be C.P. and anhydrous and the iodine should be C.P. and resublimed. The ketone may be pure or of practical grade. The materials should be so handled as to insure against contamination and to protect the same against moisture. To these ends, the iodide and the iodine should be stored, prior to use, in closed containers in a desiccator or the like and, when handled, as for weighing or the like, should be placed on glass or the like to avoid any possible metallic contamination. The finished liquid electrolyte, where stored, should be kept in sealed glass or the like containers and, if the latter are stored in air, it is advantageous that the dew point of the air does not exceed about -55 degrees F. To facilitate the maintenance of

the precautions described above, it is, in general, advisable to work with small batches of the materials.

In preparing the electrolyte solutions, a good operating technique comprises, for example, in an illustrative case, placing 2.5 grams of calcium iodide in an open, small mouth container of about 60 ml. capacity which previously has been cleaned and dried and which can easily be sealed. The container and its contents of calcium iodide is then placed in a vacuum heating chamber and evacuated to about 25 inches of mercury and heated to approximately 150 degrees F. for about 30 minutes. Promptly upon removal of the container from the vacuum chamber, 6 grams of iodine crystals are placed in said container, and then 25 ml. of diisopropylketone and 25 ml. of diisobutylketone are added to the container and the ingredients are thoroughly mixed to effect solution of the calcium iodide and iodine. The container is then sealed until the electrolyte solution is ready to be used.

In use, the interior of the resistor casing into which the electrolyte is introduced is thoroughly washed with a ketone, for example, diisobutylketone, using several rinses. The devices are placed in a vacuum heating chamber, evacuated to about 25 inches of mercury, and heated to about 150 degrees F. for about 30 minutes. The device is placed in a suitable leveling fixture and the liquid electrolyte is introduced into the device to the desired level by means of a hypodermic syringe or the like and the casing is then closed. The usual techniques in filling, sealing and testing the finished devices are employed.

While the invention has been described in detail, it will be understood that various modifications may be made without departing from the essential teachings set forth herein and which are delineated in the appended claims.

What is claimed as new and desired to be protected by Letters Patent of the United States is:

1. In a variable resistor which includes a closed receptacle containing an electrolyte and electrodes having a surface adapted to contact said electrolyte to provide a current-conducting path between said electrolyte and said electrodes, the improvement wherein said electrolyte is a solution, in a saturated ketone, of iodine and an alkaline earth metal iodide, wherein said alkaline earth metal iodide is present in proportions ranging from about 3 to about 10 grams per 100 ml. of said electrolyte solution, and the iodine is present in proportions ranging from about 8 to about 16 grams per 100 ml. of said electrolyte solution.

2. A variable resistor in accordance with claim 1, wherein said ketone is an aliphatic ketone.

3. In a variable resistor which includes a closed receptacle containing an electrolyte and electrodes having a surface adapted to contact said electrolyte to provide a current-conducting path between said electrolyte and said electrodes, the improvement wherein said electrolyte is a solution, in a saturated ketone, of calcium iodide and iodine, the calcium iodide being present in proportions ranging from about 4 to about 6 grams per 100 ml. of said electrolyte solution, and said iodine being present in proportions ranging from about 10 to about 14 grams per 100 ml. of said electrolyte solution.

4. A variable resistor in accordance with claim 1, wherein said ketone comprises at least one member selected from the group consisting of diisopropylketone and diisobutylketone.

5. A variable resistor in accordance with claim 1, wherein said ketone comprises a mixture of diisopropylketone and diisobutylketone in which the ratio of said ketones to each other by volume is from about 1 to 3 to about 3 to 1.

6. A variable resistor in accordance with claim 1, in which said ketone is a mixture of diisopropylketone and diisobutylketone and in which the ingredients of said elec-

trolyte are present in the following amounts relative to each other:

|                             |       |       |    |
|-----------------------------|-------|-------|----|
| Diisopropylketone           | ----- | ml    | 50 |
| Diisobutylketone            | ----- | ml    | 50 |
| Alkaline earth metal iodide | ----- | grams | 5  |
| Iodine                      | ----- | do    | 12 |

7. A variable resistor in accordance with claim 2, wherein said iodide comprises magnesium iodide.

8. A variable resistor in accordance with claim 2, 10 wherein said iodide comprises barium iodide.

9. A variable resistor in accordance with claim 2, wherein said iodide comprises strontium iodide.

References Cited in the file of this patent

UNITED STATES PATENTS

|           |           |       |                |
|-----------|-----------|-------|----------------|
| 2,387,313 | Wilson    | ----- | Oct. 23, 1945  |
| 2,764,653 | Schoeppel | ----- | Sept. 25, 1956 |

OTHER REFERENCES

Chem. Abstracts 47, 1953, p. 27.